

April 30, 1935.

W. W. EITEL ET AL

**1,999,806**

### OXIDE COATED CATHODE

Filed Feb. 25, 1933



INVENTORS,

JACK McCULLOUGH

BY Donald Whippincott

*ATTORNEY*

## UNITED STATES PATENT OFFICE

1,999,806

## OXIDE COATED CATHODE

William W. Eitel, San Bruno, and Jack McCullough, Palo Alto, Calif., assignors to Heintz & Kaufman, Ltd., San Francisco, Calif., a corporation of Nevada

Application February 25, 1933, Serial No. 658,524

## 4 Claims. (Cl. 250—27.5)

Our invention relates to an oxide-coated cathode for thermionic tubes, and more particularly to such a cathode which has been formed into a predetermined shape by a stretching or deforming process after the oxide layer has been applied.

Among the objects in our invention are: To provide an oxide-coated filament or cathode of high efficiency; to provide a method of preforming an oxide-coated filament to a predetermined shape before insertion into a thermionic tube; to provide a thermionic tube having a stretched oxide-coated filament; and to provide a relatively rigid pleated ribbon filament having an oxide coating which will maintain its shape under operating conditions in a thermionic tube.

Other objects of our invention will be apparent or will be specifically pointed out in the description forming a part of this specification, but we do not limit ourselves to the embodiment of our invention herein described, as various forms may be adopted within the scope of the claims.

Referring to the drawing:

Figure 1 is a longitudinal view of a thermionic tube embodying this invention, the envelope being cut away to expose the electrodes.

Figure 2 is a sectional view taken as indicated by the line 2—2 in Figure 1.

Figure 3 is a view in elevation of a device used for cold stretching and forming the cathode to a predetermined shape.

When oxide-coated filaments were first developed, a core material of platinum was commonly used, and oxides, usually a mixture of barium and strontium, were baked on to the core in a plurality of layers. Later nickel was substituted for platinum, but in all cases after coating the core material could not be deformed, as the bond between the oxide layer and the core was poor, and the oxides would flake off. Nickel, and its alloys, or other similar core materials anneal and become soft during the process of baking on the oxides, and when the completed cathode is mounted in a thermionic tube in such a condition, it is limp, lacks rigidity, and will stretch under spring tension. In addition, the annealed cathodes when self-supported either wholly or partially, in a position where the force of gravity may act on them, will gradually sag due to this stretch.

Any serious attempts heretofore to preform the filament after the oxide coating has been applied have been failures, as the oxide coating would scale off the core when the core was distorted. In certain cases, such as the bend at the top of

the usual type of hairpin filament, this cracking off did no harm and could be tolerated, as the loss of emitting material did not occur in the active portion of the filament. In other cases the completed filament could not be formed at all after the oxide coating was put on and recourse was had to forming the core into the desired shape, dipping the formed core into a solution of oxides and baking the formed cathode. This still left the formed filament in an annealed and soft condition, and the formed filament had to be handled and mounted with extreme care to prevent peeling of the oxides.

We have found that oxide-coated filaments having a dense adherent coating such as that described in the application of Jack McCullough, Serial No. 614,629, filed May 31, 1932, do not peel, flake or otherwise lose their oxide coating when the core is distorted, and this invention broadly speaking comprises providing a core, preferably of nickel, with a coating or layer of oxides as described in the above-mentioned application, and then stretching and bending the completed filament over a form to harden and set the filament into a predetermined shape, the shape here shown being a pleated ribbon.

In the drawing, which illustrates a thermionic rectifier tube as an example of one use of this invention, the customary envelope 1 is closed at one end by a reentrant stem 2 through which are sealed two cathode leads 4 and which supports, in this case, three dummy supports 5. A pleated ribbon filament 6 is welded at its ends to the cathode leads, and the cross bar of every other pleat is supported by refractory support wires 7 loosely looped around the bars. These support wires space the pleats at equal distances apart and prevent vibration of the complete filament.

An anode 9 is sealed through a projection 10 in the upper portion of the envelope, and the exterior anode lead is connected to an anode cap 11. A base 12 is sealed on the stem end of the envelope, and the two cathode leads are connected to cathode prongs 14 insulated from the base by washers 15.

The cathode is prepared for insertion in the tube by first coating a core, preferably of nickel ribbon with an adherent layer of oxides, or similar electron-emitting material, and preferably by the use of the method and material disclosed in the above-mentioned application of Jack McCullough.

The coated ribbon is then stretched and bent into a predetermined form, preferably while cold,

by the use of the stretching and forming device shown in Figure 3.

A foundation bar 16 is provided with two round studs 17, one at each end, and is drilled and tapped in the center to receive a screw 19, provided at its outer end with a knurled handle 20, and at the other end with an unthreaded projection 21, separated from the threads of the screw by a shoulder 22. A movable bar 23 is drilled to slide over the studs 17 and also to receive the projection 21. A retainer collar 24 is then passed over the end of the projection 21 and fixed in place by pin 25. The movable bar will then slide on the studs in response to the turning of the screw 19.

Each stud is provided with an adjustable stop 26 and a terminal nut 27.

Equally spaced along each bar are ribbon pins 29, those on the foundation bar being preferably offset in position from those of the movable bar. Removable split pins 30 are positioned at one end of one bar and at the opposite end of the other bar. These pins are preferably tapered to grip the ribbon.

One end of the coated ribbon is placed in one split pin and the pin driven into its hole to grip the ribbon securely.

The ribbon is then wound loosely around alternate pins, first on one bar and then on the other, and the free end of the ribbon secured in the remaining split pin. The screw is then rotated to take up the slack, and then further rotated to stretch the ribbon. The adjustable stops 26 are so positioned that given lengths of ribbon may be uniformly stretched, and to prevent stretching beyond the elastic limit of the core material.

The tension is then relieved, the split pins removed, and the finished pleated filament removed from the frame. It will be found that the core material has been hardened by the stretching and bending process, and that the filament has become set into the form defined by the location and number of the pins. The formed filament may then be handled without excessive care, and mounted on the cathode leads.

It may be desirable, however, to use the stretching frame as a holder for the filament, and the filament may be welded to the cathode leads while still on the frame, and then removed.

The finished stretched and set filament when used in a thermionic tube does not tend to sag or further deform in use, and much more precisely shaped cathodes may be fashioned than when

annealed ribbons are used. The emitting properties of the stretched filament have not been diminished by the stretching process, but on the contrary there appears to be some evidence of an increased efficiency, the reason for which we are 5 not at present able to state.

It is well known that bending as well as stretching will harden and set a metal. In the stretching frame as described, the bars of the pleats are stretched, but the end loops are bent rather than 10 stretched, although the outer circumference necessarily has to be stretched to form the bend. It is therefore possible to carry out the spirit of the invention by bending alone, as such bending will give the same result as longitudinal extension. 15 This feature is of great financial advantage in the formation of cathodes from sheet core material, as for example the cylindrical cathodes for heater type electron tubes. The usual procedure is to blank and form the core material, mount 20 and finally coat and bake on the oxide layer. Our invention permits the coating to be done first on the sheet stock, the blanking and forming into a cylinder being done after the oxide layer has been applied. The forming into a cylinder will 25 harden the core material and give all the advantages here disclosed for a ribbon type filament.

We claim:

1. The method of forming an electron-emitting cathode, which comprises coating a metallic ribbon with an adherent layer of electron-emitting material, and subsequently cold stretching said ribbon throughout its length into the desired form. 35

2. The method of forming an electron-emitting cathode, which comprises coating a ductile ribbon with an adherent layer of electron-emitting oxides, and subsequently cold stretching all of said ribbon into the desired form. 40

3. The method of forming an electron-emitting cathode which comprises coating a metallic core with an adherent layer of electron-emitting material, and subsequently deforming all of said core into the desired shape. 45

4. The method of forming an electron emitting cathode which comprises coating an elastic metallic core with a non-elastic layer of electron emitting material and subsequently cold stretching all of said core into the desired form. 50

WILLIAM W. EITEL.  
JACK McCULLOUGH.